

June 28, 1927.

1,633,787

O. KRESS

OIL AND GREASE PROOF PAPER AND CONTAINER MADE THEREFROM

Filed Aug. 1. 1925



Patented June 28, 1927.

1,633,787

# UNITED STATES PATENT OFFICE.

OTTO KRESS, OF APPLETON, WISCONSIN, ASSIGNOR TO AMERICAN LAKES PAPER COMPANY, OF CHICAGO, ILLINOIS, A CORPORATION OF DELAWARE.

## OIL AND GREASE PROOF PAPER AND CONTAINER MADE THEREFROM.

Application filed August 1, 1925. Serial No. 47,439.

The present invention has primarily for its object the provision of an improved composite paper sheet adapted to carry oils, lard, grease, and like materials, and to provide an efficient and inexpensive container made therefrom, whereby such materials as gasoline, lubricating oil, lard, grease, or the like may be carried, the container being of such cheap construction that after it has been used once it may be discarded.

I have discovered that it is possible to render sheets of paper impermeable to the passage of oils and grease if such sheets are united together by a non-drying cement, insoluble in oil and carrying water in sufficient quantity to prevent the passage of oil therethrough, this being due to the fact that the water carried by the cement repels the passage of oil and grease. I have found also that a container made from sheets of paper so united together will for a long period of time effectively serve to retain oils, grease, or the like, the water carried by the cement that unites the sheets repelling the oil or grease, which otherwise would pass through the pores of the paper.

The invention consists in the features of novelty hereinafter described, illustrated in the accompanying drawing and particularly pointed out in the claims at the end of this specification.

Figure 1 is a sectional view showing a composite paper sheet formed of two sheets of paper united together in accordance with my invention; Figure 2 is a perspective view showing a bag-shaped container embodying my invention; Figure 3 is a sectional view showing a plurality of sheets of paper united together by an oil and grease proof cement, these sheets being given greater body by having united thereto a sheet of paper board; Figure 4 is a perspective view of a container in the form of a box or carton made from the composite sheet illustrated in Fig. 3 of the drawing; Figure 5 is a sectional view similar to Fig. 1, but having a paper sheet united thereto by waterproof cement; and Figure 6 is a view similar to Fig. 3, with an additional sheet of paper united thereto by a waterproof cement.

Referring to Figs. 1 and 2 of the drawing,

A and B designate two sheets of paper and C denotes a thin film of adhesive material whereby the sheets will be inseparably united together. The sheets of paper A and B may be of any suitable character or quality, although I prefer to employ so-called "grease-proof" papers, such as are known in the trade under the names of "grease proof", "glassine" and "vegetable parchment." In preparing the composite sheet illustrated in Fig. 1, I prefer to apply the adhesive to the opposing surfaces of two sheets A and B, in order to be absolutely sure of a continuous film of such adhesive over the sheets, although if desired, the adhesive C may be applied to the surface of one sheet of paper only and the other sheet may be then firmly pressed thereon. While I regard it within the broad scope of my invention to employ for uniting the sheets of paper any suitable cement or adhesive that will carry water in sufficient quantity to prevent the passage therethrough of oil or grease, one preferred adhesive which gives very satisfactory results consists of a strong solution of commercial glucose which may be varied in concentration from 40 to 70% of actual weight of dry glucose; that is to say, the solution may contain from 60 to 30% of water. In order to render the film more flexible, there may be added, if desired, from 5 to 30% of glycerine, which will serve to maintain the film in moist condition and prevent the evaporation of the water for a long period. If desired, also, there may be added to the glucose solution from 5 to 30% in weight of dry calcium chloride, as this salt is very hygroscopic and will tend to draw moisture and so maintain the water content of the adhesive for a long period. An adhesive such, for example, as that above described, will be found to be insoluble in oil and to carry water in sufficient quantity to prevent the passage of oil therethrough, and is, in effect, non-drying. By the term "non-drying", I mean that the adhesive is of such character that the moisture thereof will not evaporate or dry out for a long period of time.

The composite sheet of paper such as illustrated in Fig. 1 of the drawing may be made

up into a variety of forms of containers for oils or grease. In Fig. 2, the composite sheet is shown as formed into a bag-like container, the top of which is closed in any suitable manner and is provided with a filling tube D of suitable material, and having a convenient handle E whereby the bag may be carried. Bags of this character can be very cheaply made, and the material being flexible, can be conveniently stored for use. When such a bag or container is filled with oil (gasoline, for example), it will be found that while the oil will in time penetrate the interior sheet, the water carried by the film of non-drying cement or adhesive will prevent the passage of the oil through the bag. If desired, the outer surface of the bag or container may be covered with an additional sheet of paper (such as Kraft paper) pasted thereto and serving to strengthen the bag.

In Fig. 3 of the drawing is shown a composite sheet rendered somewhat heavier than the composite sheet illustrated in Fig. 1 and better adapted for forming boxes or cartons for containing lard, grease, or other oily materials. This composite sheet is shown as formed of paper sheets A and B united by a film C of oil or grease proof cement as heretofore described, a sheet of paper board A<sup>2</sup> being shown as united to the sheet A by a film A<sup>3</sup> of suitable cement, such as silicate of soda, starch paste, or the like.

In Fig. 4 there is shown a box or carton made from the composite sheet illustrated in Fig. 3. This carton may comprise a body portion of ordinary shape and construction, having end flaps at its top adapted to be turned inward after the box has been filled.

If it is desired to make the container moisture proof, as well as oil and grease proof, a further sheet of paper may be connected to the outside of the container by a thin film of asphalt cement. Thus in Fig. 5, I have shown a composite sheet similar to that illustrated in Fig. 1, but having an outer sheet A<sup>4</sup> united to the sheet of paper A by a thin film A<sup>5</sup> of asphalt. So, also, in Fig. 6 is shown a composite sheet similar to that illustrated in Fig. 3, but having an outer sheet A<sup>4</sup> united to the sheet of paper board A<sup>2</sup> by a thin film of asphalt or equivalent waterproof cement.

Figures 1, 3, 5 and 6 are necessarily exaggerated in order to show the elements comprising the composite sheets, but it will be understood that the composite sheets shown in Figs. 1 and 5 are sufficiently thin and flexible to permit the formation of bag-like containers, and the composite sheets shown in Figs. 3 and 6, while somewhat thicker and somewhat stiffer, are sufficiently flexible to form cartons or containers such as illustrated in Fig. 4.

My improved composite paper sheet will be found not only sufficiently flexible to

enable containers such as above described to be formed therefrom, but the film or films of cement employed in uniting the sheets of paper are of such non-drying, flexible character, that it will not become brittle and will not crack when the containers are folded, scored, printed upon or carelessly handled. The composite sheet illustrated in Figs. 1 and 5 of the drawing will be found particularly well adapted in the lining of boxes, barrels, or the like, that are to contain oils, solid grease, or like materials.

The details above described and the precise character and composition of the oil and grease proof cement may be varied without departure from the broad scope of the invention.

Having thus described my invention, what I claim as new and desire to secure by Letters Patent is:—

1. A composite oil and grease proof sheet comprising two sheets of paper permanently united together by a non-drying cement insoluble in oil and carrying water in sufficient quantity to prevent the passage of oil therethrough.

2. A composite oil and grease proof sheet comprising two sheets of paper permanently united together by a non-drying cement insoluble in oil and carrying water in sufficient quantity to prevent the passage of oil therethrough and having a supplemental sheet united thereto by a film of waterproof cement.

3. A composite oil and grease proof sheet comprising two sheets of paper united together by a non-drying cement consisting mainly of glucose and water.

4. A container for oil, lard, or like material comprising sheets of paper united together by a non-drying cement, insoluble in oil, and carrying water in sufficient quantity to prevent the passage of oil therethrough.

5. A container for oil, lard, or like material comprising sheets of paper united together by a non-drying cement, insoluble in oil, and carrying water in sufficient quantity to prevent the passage of oil therethrough, one of said sheets having a supplemental sheet united thereto by a waterproof cement.

6. A container for oil, lard, or like material comprising a paper board having upon one side a sheet of paper united thereto by a film of asphalt and having united to its other side at least two sheets of paper connected together by a film of non-drying cement, insoluble in oil, and carrying water in sufficient quantity to prevent the passage of oil therethrough.

7. A composite oil and grease proof sheet comprising two sheets of paper united together by a non-drying cement consisting mainly of glucose, water and calcium chloride.

8. A composite oil and grease proof sheet

comprising two sheets of paper united together by a non-drying cement consisting mainly of glucose, water, calcium chloride and glycerine.

5 9. The method of making an oil and grease proof container that consists in interposing between two sheets of paper a non-

drying cement insoluble in oil and carrying water in sufficient quantity to prevent the passage of oil therethrough, and thereafter <sup>10</sup> incorporating said sheet in the form of a container.

OTTO KRESS.